

April 18, 1961

R. C. GASMIRE

2,979,801

METHOD OF MAKING REINFORCED CAST SHAPES

Filed Sept. 11, 1958

2 Sheets-Sheet 1



INVENTOR.

RICHARD C. GASMIRE  
BY W. A. Schaeich

Leonard S. Donkin  
ATTORNEYS

April 18, 1961

R. C. GASMIRE

2,979,801

METHOD OF MAKING REINFORCED CAST SHAPES

Filed Sept. 11, 1958

2 Sheets-Sheet 2



INVENTOR.

*Richard C. GASMIRE*  
BY *W. A. Jokisch*

*Leonard S. Gorin*  
ATTORNEYS

1

2,979,801

## METHOD OF MAKING REINFORCED CAST SHAPES

Richard C. Gasmire, Toledo, Ohio, assignor to Owens-Illinois Glass Company, a corporation of Ohio

Filed Sept. 11, 1958, Ser. No. 760,381

1 Claim. (Cl. 25—154)

The present invention relates to a method of making reinforced cast shapes. More particularly, this invention proposes a method of inserting reinforcing grids into uncured cementitious bodies of the cast calcium silicate (commonly known as "cellular concrete").

Cellular concrete bodies are commercially manufactured as unit slabs having integral metallic reinforcing grids. A typical commercial casting mix is a slurry of cement, lime, and silicate to which a preformed foam is added prior to the pouring of the casting mix into a multiple mold. This mold is preferably of unit length and width dimensions but of multiple slab thickness, the mold contents being removed and subdivided into unit slabs after pre-curing at ambient pressure and temperature conditions to a self-sustaining condition. The pre-cured cast block, after severing into unit slabs, is generally autoclaved for a period of about ten hours at a steam pressure of about 150 lbs. per square inch to form a finished product having a density of about 30 to 40 lbs. per cubic foot.

The present invention proposes the insertion of spaced reinforcing grids into the cast multi-slab block at unit-slab spaced intervals after the slurry or casting mix has been poured into the mold, but prior to the pre-curing of the casting mix. Since the casting mix is quite fluid when poured into the mold (to promote fluid handling of the mix and to insure complete filling of the mold), some means must be provided for holding the grids in position within the casting mix. Inasmuch as the multi-slab block is severed lengthwise into several slabs, the reinforcing grids must be quite accurately positioned and retained in spaced parallel relation.

In accordance with the present invention, each reinforcing grid is secured to a plurality of longitudinally spaced hangers which project vertically into the mold. These hangers are preferably each in the form of a vertically extending rod secured to the reinforcing grid by a frangible connection, as by a tack weld, and provided with an abutment for contacting a positioning means superimposed over, but lying outside the confines of, the casting mold. Since the hanger rods are cylindrical in shape and are only lightly secured to the reinforcing grids, the hanger rods can be rotated to break their connection with the reinforcing grid, and then the hanger rods can be retracted vertically out of the pre-set casting mix after the casting mix has solidified sufficiently to retain the reinforcing mesh in position, but prior to integration of the hanger rods into the mix-mesh assembly.

The method of the present invention involves the suspension of the reinforcing mesh in the slurry-filled mold by means of the supporting rods, effecting relative movement between the supporting rods and the mesh after the slurry has been sufficiently solidified to prevent displacement of the mesh, and the retraction of the supporting rods from the at least partially solidified casting mesh.

It is, therefore, an important object of the present invention to provide an improved method of making reinforced cast shapes by the insertion of a reinforcing mesh

2

into an uncured casting slurry, supporting the mesh in position within the slurry until the slurry has solidified sufficiently to retain the mesh in position, and then retracting the mesh support from the slurry.

- 5 It is a further object of this invention to provide a method for inserting a reinforcing mesh into an uncured cementitious body which is subsequently cured to a self-sustaining state by vertically suspending the mesh from an attached suspending means in the uncured body, at 10 least partially curing the body, detaching the suspending means from the mesh, and removing the mesh suspending means.

Other objects and advantages of the invention will appear from the following detailed description taken in conjunction with the annexed drawings, in which:

On the drawings:

Figure 1 is an elevational perspective view of a cast slab having an integrally cast reinforcing mesh, the slab being made in accordance with the method and apparatus 20 of the present invention;

Figure 2 is a sectional view taken along the plane 2—2 of Figure 1;

Figure 3 is a plan view of an apparatus of the present invention;

25 Figure 4 is a sectional view taken along the plane 4—4 of Figure 3; and

Figure 5 is a sectional view taken along the plane 5—5 of Figure 3.

As shown on the drawings:

- 30 In Figs. 1 and 2, reference numeral 10 refers generally to a cast calcium silicate slab having an integrally cast metallic reinforcing grid 11 disposed interiorly thereof. It will be noted that the slab 10 presents continuous exterior surfaces and that the reinforcing mesh 11 is disposed wholly interiorly thereof. The mesh 11 comprises horizontal rods 12 and vertical rods 13 welded or otherwise secured to one another at their points of intersection and the upper and lower marginal extremities of the grid 11 are deflected laterally and vertically to provide offset 35 end portions 14 (best shown in Figure 2) which aid in securing the mesh in position within the slab.

As best illustrated in Figures 3, 4 and 5, the slab 10 is made in a mold 20 which comprises a plane mold bottom 21 having superimposed thereon side walls 22 and 40 end walls 23, the walls being secured to one another and to the bottom wall by suitable means, such as swing bolts 24.

When the mold walls 21, 22 and 23 are assembled as 45 illustrated in Figures 3, 4 and 5, the walls define an interior molding space 25 which is adapted to receive a casting mix. This casting mix comprises water, cementitious ingredients, pozzolans, accelerators, and foam or foam-forming ingredients.

The cementitious ingredients are preferably cement 50 of the Portland type, either normal or of the high early strength type, and lime, preferably quick lime, although a high calcium hydrate of lime may be utilized. Any pozzolanic material may be utilized, a pozzolan being defined as a finely divided material rich in silica or alumina 55 which, while not necessarily cementitious in itself, will react at ordinary temperatures with hydrated lime in the presence of water to form insoluble cementitious products. The preferred pozzolan is silica flour, although ground silica sand, burned oil-shell, fly ash, ground brick or tile, volcanic ash, granulated slag, diatomaceous earth, 60 pomace dust, glass grinding waste, or other suitable pozzolans may be utilized.

70 Preferably, a pre-formed foam is utilized, the foam being introduced into the cementitious slurry after the remainder of the slurry has been formed. Foaming agents of the following type may be used: detergents, resin soap, saponin, alkylated naphthalene, sulphonates,

neutralized synthetic resins or hydrolyzed protein, or commercial foaming liquids, such as National Cote HT-1 manufactured by National Foam Systems, Inc., of Westchester, Pennsylvania.

To form a typical casting slurry for use in forming foam concrete, the following composition may be utilized:

|                   | Percent |
|-------------------|---------|
| High Early cement | 28.6    |
| Silica flour      | 66.5    |
| Quick lime        | 4.9     |

Calcium chloride may be added as an accelerator, preferably to an extent equal to about 2% by weight of the cement content of the slurry dry ingredients.

To form the slurry, the dry ingredients are mixed with an amount of water sufficient to yield a water-to-solids ratio of about 0.75 by weight and to yield a cementitious slurry having a wet density of about 46 pounds per cubic foot. A commercial foaming agent sold under the trade name "National Foam Liquid" manufactured by National Foam Systems, Inc., of Westchester, Pennsylvania, and consisting of a 3% solution of the foaming agent and water and sufficient air to form a consistent air-stable foam as utilized to an extent consisting of 0.016 gallon of foaming agent per 100 pounds of slurry.

The slurry is introduced into the mold space 25 and allowed to air cure. As introduced into the space 25, the slurry is readily flowable and is obviously incapable of supporting the vertically disposed wire reinforcing mesh 11 therein.

Also, it will be noted from Figures 3 and 5, the space 25 is of multi-slab dimensions, i.e., the height of the mold space is substantially equal to the width of the individual slabs, and the length of the mold space is substantially equal to the length of the individual slabs. However, the mold space is of multiple slab thickness. Because of the dimensions of the mold space and the fluidity of the slurry introduced thereto, it is necessary to suspend a plurality of the wire meshes 11 within the slurry-mesh filled space.

As best illustrated in Figures 4 and 5, there is secured to each mesh 11 a vertically extending support rod 30. More particularly, from Figure 5 it will be seen that each of these supporting rods 30 is secured to the associated mesh 11 adjacent the upper and lower extremities of the mesh, for example as at 31. Preferably, the rods 30 are secured to the mesh by tack welding or otherwise lightly or frangibly securing the rod against the back face of the reinforcing mesh, i.e., against that face away from the bent ends 14 thereof.

Further, it will be noted that each of the rods has secured thereto a locating abutment 32 adjacent the upper extremities of the rods and outside the confines of the mold space 25. This abutment 32 preferably is an enlarged washer which is securely welded or otherwise fastened to the rod 30. Superimposed over the mold space 25 are a pair of longitudinally spaced locating jigs 40, each of these jigs comprising upper and lower transversely extending support plates 41 and 42 secured together in vertically spaced relation by spacers 43, and each of the plates 41 and 42 are provided with spaced longitudinally elongated notches 44 of such size as to

slidably receive therein the upper extremities of the rods 30 projecting above the mold space 25. It will be noted that the notches of both of the jigs 40 open in the same direction and it will be appreciated that these notches 5 make possible the ready assembly of the jigs 40 and rods 30 as illustrated in Figures 3-5.

The manipulative steps involved in practicing the method of the present invention include securing of the support rods 30 to the reinforcing mesh 11. The mesh together with the lower extremities of the reinforcing rods are submerged within the body of slurry filling the mold space 25. The jigs 40 are now superimposed over the mold space, contacting the side walls 22 of the mold and the jigs are slid into position beneath the abutments or washers 32. Next, the mesh is adjusted longitudinally 15 within the mold space to bring the individual grids into accurate transverse alignment. The transverse spacing of the notches 44 in the plates 41 and 42 insures the accurate transverse spacing of the grids adjacent thereof. 20 Next, the slurry is pre-cured preferably at ambient temperatures and pressures with the mesh grids 11 and the suspension rods 30 in situ. After the slurry has been pre-cured and sufficiently solidified to retain the mesh grids 11 in position, the suspension rods 30 are rotated 25 slightly to break the tack welds 31, thereby separating the suspension rods from the associated grids. The suspension rods are then removed vertically from the body of the at least partially solidified slurry, and the mesh grids are isolated within the solidified slurry filling the 30 mold space.

After removal of suspension rods 30, the slurry is further pre-cured, if necessary, to a completely self-sustaining state and the mold side and end walls 22 and 23 are removed from the pre-cured block of multi-slab 35 thickness. The cast block is then severed longitudinally along unit slab thickness planes as, for example, described and claimed in United States Patent No. 2,957,223, granted October 25, 1960, to Joseph C. Hamilton, and assigned to the assignee of the present invention. 40

#### What is claimed is:

The method of locating a reinforcing wire mesh grid within a cast calcium silicate slab comprising the steps of casting a curable cellular concrete slurry into a mold, tack welding a plurality of smooth elongate cylindrical suspension rods to a wire mesh grid to project vertically from said mold when said grid is at the desired location within said slurry, immersing said grid into the slurry and supporting the projecting portions of said suspension 45 rods to support said grid at the desired location within said slurry, partially curing the slurry to an extent sufficient to support said grid, rotating each suspension rod relative to the grid about its vertical axis to rupture the tack welds, and withdrawing each suspension rod from 50 said slurry in a direction along its vertical axis.

#### References Cited in the file of this patent

#### FOREIGN PATENTS

|    |         |               |                |
|----|---------|---------------|----------------|
| 60 | 522,231 | Belgium       | Sept. 15, 1953 |
|    | 839,922 | Germany       | May 26, 1952   |
|    | 291,838 | Great Britain | June 5, 1928   |